

## UNITED STATES PATENT OFFICE.

ADAM CHARLES GIRARD, OF PARIS, FRANCE.

## PROCESS OF MAKING EXPLOSIVES.

SPECIFICATION forming part of Letters Patent No. 663,166, dated December 4, 1900.

Application filed February 3, 1900. Serial No. 3,824. (No specimens.)

*To all whom it may concern:*

Be it known that I, ADAM CHARLES GIRARD, a citizen of the Republic of France, residing at Paris, France, have invented certain new and useful Improvements in or Relating to the Manufacture of Explosives, (for which I have made application for Letters Patent in France on the 30th of December, 1899, under No. 295,754, and in Great Britain on the 3d day of January, 1900, under No. 214,) of which the following is a specification.

Vegetable and animal oils used in the manufacture of chlorate explosive powders cannot be employed alone with chlorate and perchlorate, because in order to obtain a sufficiently strong explosion the oil must be added to the body supporting combustion in such quantity that it (the oil) will exude. In former patents it has been stated that the solubility of nitro and azo derivatives in oil permitted the oil to be solidified while increasing its power and providing the explosive with advantageous properties, thus producing a substance which is solid when cold and liquid at a higher temperature.

In the course of my investigations I have found that other bodies, such as soaps, are capable of solidifying vegetable and animal oils and rendering them suitable for the manufacture of chlorate and perchlorate explosives by diminishing at will the quantity of the nitro and azo derivatives and by leaving out such substances altogether. Leaving out these substances slightly diminishes the effectiveness and the bursting power of the explosive; but as, on the other hand, it reduces the cost of manufacture it is useful to have an explosive less powerful, but also cheaper. This process of solidification of the oil permits, moreover, both the effectiveness and properties of the explosive to be varied almost at will, thereby rendering it suitable for all the various requirements as regards industrial uses. This solidification of the animal or vegetable oils is effected by the dissolution of a soap having either potash or soda as its base, the soap being manufactured with an animal or vegetable oil, or even with resin. The soap employed should be first dried at a temperature of between 120° and 130° centigrade, so as to drive out as much liquid or humidity as possible. The dried soap is added to the oil in the proportion of from ten to fifteen per

cent. The mass is then thoroughly stirred and heated for two or three hours at a temperature between 150° and 170° centigrade. The whole of the soap will not dissolve. Consequently it will be necessary to filter the mass. In such case the operation of filtering must take place at a temperature at which the solidified oil is rendered liquid, which temperature depends on the nature of the oil employed. In the case of ricinie or castor oil, for instance, such filtration may be effected at a temperature of between 105° and 115° centigrade. The filtered product is almost solid and of a consistency varying between that of vaseline and paraffin. It does not run at the ordinary temperature, not even at a temperature of 40° centigrade. To this substance may very easily be added at a temperature of 80° centigrade the material to support combustion in the form of powder. This mass after cooling is very plastic and can be easily introduced into the mining-holes, where it fills all the space and does not run out. It is possible to dissolve in this solidified oil nitro and azo derivatives, nitrated ethers—such as nitrate of amyl, nitroglycerin, nitrocellulose, and nitromannites—which dissolve in the solidified oil in the manner of nitrate derivatives, as in oil not so treated, and the solution when cold is simply slightly more consistent in the case of solidified oil than in that of the ordinary oil. Acid derivatives may not be added to such oil without reducing it to its original condition. Thus picric acid, for instance, forms an alkaline picrate in the oil, which thereby is reduced to almost its original condition; but picrates which have no reaction may be added to it. In such oil a variety of combustible bodies may be incorporated—such as starch, cellulose, dry pitch, resin, wood-charcoal, and sulfur—with or without nitro and azo derivatives, and also supporters of combustion, such as alkaline chlorates, perchlorates, nitrates, and the like.

Below are given several formulæ of explosives with solidified oil:

First. Chlorate of potassium, eighty parts; solidified oil, twenty parts.

Second. Perchlorate of ammonium, eighty parts; solidified oil, twenty parts.

Third. Chlorate of potassium, eighty parts; nitronaphthalene, six parts; solidified oil, fourteen parts.

Fourth. Perchlorate of potassium, seventy-five parts; solidified oil, sixteen parts; nitro-naphthalene, four parts; picrate of potassium, two parts.

5 Fifth. Chlorate of potassium, eighty parts; solidified oil, sixteen parts; azobenzol, four parts; picrate of potassium, two parts.

While in the following claims a chlorate or perchlorate is mentioned as the supporter of combustion, other equivalent substances, such as specified, may within the scope of the invention be employed with like results. In the same manner while nitronaphthalene is mentioned in the claims as the combustible body employed it will be evident that other equivalent substances, such as specified, may within the scope of the invention be employed with similar results.

What I claim as my invention, and desire 20 to secure by Letters Patent, is—

1. In the manufacture of explosives, the process consisting in solidifying an oil by dissolving therein a suitable soap, and then adding a chlorate to support combustion.

2. In the manufacture of explosives, the 25 process consisting in solidifying an oil by dissolving therein a suitable soap, then adding a chlorate to support combustion, and nitronaphthalene as a combustible body.

3. In the manufacture of explosives, the 30 process consisting in solidifying an oil by dissolving therein a suitable dry soap, then adding a chlorate to support combustion, and nitronaphthalene as a combustible body.

4. In the manufacture of explosives the 35 process consisting in solidifying the oil employed in such manufacture by adding dry soap thereto and heating the mixture, then filtering the liquid product and adding a chlorate to support combustion.

In testimony whereof I have signed my name to this specification in the presence of 40 two subscribing witnesses.

ADAM CHARLES GIRARD.

Witnesses:

EDWARD P. MACLEAN,  
EMILE LEDREL.